

Jan. 2, 1962

L. A. L. ESSELING

3,015,761

SEMI-CONDUCTIVE ELECTRODE SYSTEM

Filed June 27, 1958



Fig. 1



Fig. 2



Fig. 3

INVENTOR  
LUDOVICUS AUGUSTINUS LAMBERTUS ESSELING

BY  
*Frank R. Jinfen*  
AGENT

# United States Patent Office

3,015,761  
Patented Jan. 2, 1962

1

3,015,761

SEMI-CONDUCTIVE ELECTRODE SYSTEM  
Ludovicus Augustinus Lambertus Esseling, Nijmegen,  
Netherlands, assignor to North American Philips Com-  
pany, Inc., New York, N.Y., a corporation of Dela-  
ware

Filed June 27, 1958, Ser. No. 745,032  
Claims priority, application Netherlands July 1, 1957  
9 Claims. (Cl. 317—234)

This invention relates to semi-conductor devices, for example transistors or crystal diodes, having a semi-conductive body to which one end of at least one electrode wire is secured by fusion.

It has previously been suggested for the body, together with a wire applied thereto at one end, to be heated at a temperature such that both elements fuse together at the contact area.

When it is endeavoured in this way to secure by fusion a wire of aluminum, it appears, more particularly if the semi-conductive body consists of silicon, that heating above the melting point of aluminum is necessary, so that the wire, although it is covered with a natural oxide layer, flows together into a drop or at least loses its filamentary form. Electrodes of aluminum are therefore manufactured by applying by fusion either pellets or thin discs of aluminum. However, it is difficult for the resultant electrodes to be provided with supply wires, since, as is well-known, soldering to aluminum is in practice impossible as a result of the aforementioned natural oxide layer, which spontaneously forms on aluminum due to action of the oxygen in the air.

An object of the invention is inter alia to provide a construction in which these disadvantages do not occur, and also a method by which this construction may be realized in a simple manner.

According to the invention, the wire of which at least the envelope consists of aluminum, has so thick a genetic oxide layer on its cylindrical outer surface that fusion of the aluminum is possible without breakage of the oxide layer.

Said oxide layer preferably has a thickness comprised between 5 and 40 microns. Consequently, this layer is much thicker than the natural oxide layer already present on aluminum and which has a thickness of only 0.1 to 0.2  $\mu$ .

An oxide layer of sufficient thickness may be obtained in a simple manner by chemical means or by anodic oxidation.

The method according to the invention is characterized in that a wire, of which at least the envelope consists of aluminum, is provided with a genetic oxide layer of a thickness such that fusion of the aluminum is possible without breakage of the oxide layer, whereupon one end of this wire is secured by fusion to a semi-conductive body. It will be evident that it is also possible for short pieces to be cut from a long oxidized wire.

It is to be noted that a genetic oxide layer is to be understood to mean a layer, the aluminum content of which substantially originates from the initial wire. The term "oxide layer" is to be understood to mean also layers consisting of oxide hydrates, such as the compound  $Al_2O_3 \cdot H_2O$ , and furthermore oxide layers strengthened by impregnation or in another way, as will be discussed more fully hereinafter.

As a rule, the wire homogeneously consists of aluminum. However, it is possible to utilize a wire having an envelope of aluminum and a core of a different material. During fusion, the envelope and the core may fuse together.

The core may consist, for example, of semi-conductive material, such as germanium or silicon. Its presence in

2

the electrode material, in the present case in the wire, may restrict penetration of the electrode material into the semi-conductive body in a manner known per se. Such a wire may be manufactured by filling an aluminum tube with the other material and subsequently reducing the cross-section of the whole by swaging or expanding.

In order that the invention may be readily carried into effect, several embodiments will now be explained in detail, by way of example, with reference to the accompanying drawing, in which:

FIG. 1 shows diagrammatically a side-view of a diode;

FIG. 2 shows a device for applying wires to semi-conductive bodies by fusion.

FIG. 3 is a cross-sectional view of a semi-conductor device according to the invention.

The diode shown in FIG. 1 comprises a thin silicon disc 1 of conductivity, to which an aluminum wire 2 is secured by fusion in an oven at a temperature preferably higher than the melting point of aluminum, for instance 800° C. The oven temperature may however in principle be lower than the melting point of aluminum, but higher than the eutectic temperature of the silicon-aluminum mixture. The heating takes place in reducing surroundings, for example in a mixture of nitrogen and hydrogen. A small addition of hydrochloric-acid gas as a flux enhances adhesion of the wire to the body. The wire is provided with a genetic oxide layer 3 which ensures that the form of the wire substantially does not change during heating and that flowing-out of the aluminum is restricted within certain limits. The strengthened oxide layer is naturally not present at the area where the aluminum must fuse together with the silicon. The reducing atmosphere does not or not greatly affect the oxide sheath. The thickness of the wire is not essential to the invention and is usually from 100 microns to several millimetres in practice.

The semi-conductive body is secured to a base 5 by means of tin solder 4.

The use of a flux, such as hydrochloric-acid gas, is greatly simplified due to the presence of the oxide layer, since such fluxes usually also chemically attack the aluminum to a considerable extent, which phenomenon is greatly suppressed by the presence of the strengthened oxide layer.

The aluminum wire with its strengthened oxide layer may be manufactured in various ways known per se, that is to say by purely chemical means or an anodic oxidation. The last-mentioned method usually gives thicker oxide layers than the first-mentioned and is therefore preferable for comparatively thick wires.

One example of each method will now be given hereinafter.

I

Pure aluminum wire is degreased for half a minute in a bath containing 15 gms. of sodium hydroxide to 100 gms. of water at a temperature of 20° C. After rinsing in water, any residues of this bath are neutralized in a solution of nitric acid having a specific gravity of 1.25 at room temperature for 1 minute, whereafter the wire is rinsed in water. Such removal of grease is not necessary for wire which is very clean.

Subsequently, the wire is dipped for 4 minutes in an oxidizing bath of the conventional type containing for example,

55 ccs. of phosphoric acid  $H_3PO_4$ , density 1.7

22 gms. of chromic acid  $CrO_3$

3.3 gms. of acid ammonium fluoride  $NH_4HF_2$

2.2 gms. of acid diammmonium phosphate  $(NH_4)_2HPO_4$

1000 gms. of water

at a temperature of 50° C. Of course also other oxidizing baths can be used.

The wire is then carefully rinsed and dried. The thickness of the oxide layer is from 3 to 5 microns.

Aluminum wire degreased as described in Example I is subjected at 20° C. to an anodic treatment at 60 volts (direct voltage) for one hour. The bath was a conventional one, containing 50 gms. of oxalic acid  $C_2H_4H_2O$  per litre. Also other oxidizing baths are suitable. The thickness of the resultant oxide layer was about 40 microns.

Several such purely chemical or electro-chemical methods are known and it is not essential to the invention which method is used, provided the resultant layer has sufficient thickness and, of course, does not contain constituents detrimentally affecting the performance of the semi-conductor device.

From the oxidized wire obtained in accordance with Example I or II, there are cut off pieces 10 each having a length of 15 mms., which in a jig of graphite are placed on the bodies of silicon (see FIG. 2). The jig is constituted by two parts 11 and 12, which fit into each other. The part 12 has recesses 13, by which the semi-conductive bodies are kept in position, and perforations 14, by which the pieces of wire 10 are centred with respect to the bodies.

After the above-described heating in an oven, the pieces of wire are found to have retained their initial form. Subsequently, the semi-conductive bodies are after-etched in the usual manner, for example with the use of hydrofluoric acid, the strengthened oxide-layer then again having the advantage of protecting the aluminum itself against chemical attack.

It is to be noted that the pieces of wire 10, before being applied by fusion, are preferably provided with a flat end by polishing or filing.

The pieces of wire 10 may be connected by spot-welding to a piece of copper wire or copper cable which may be connected by soldering to a connecting member.

During spot-welding, the strengthened oxide layer is naturally broken through, but this is not dangerous, the operation being effected at some distance from the semi-conductive body.

FIG. 3 shows an example of such a structure applied to a diode in an evacuated envelope. The envelope comprises a base 30 with a threaded stud 31 for attachment, and a cap 32. The cap 32 contains a glass lead-through insulator 33 containing a small metallic tube 34. The silicon body 1 is soldered to the base 30, whereas the aluminum wire 10 is secured by spot-welding to a copper wire 36 at 35. After this wire has been passed through the tube 34, the base 30 and the cap 32 are secured together by means of flanges 37 and 38, for example by welding. Subsequently, the envelope is fully closed due to the copper wire 36 being soldered in the tube 34.

As previously mentioned, it is alternatively possible to utilize a wire having an envelope of aluminum and a core of different material. The latter may contain or consist of an active impurity such as a donor and/or an acceptor, but also semi-conductive material and more

particularly the same material as that of the body to which the wire is secured.

What is claimed is:

- 5 1. An electrode comprising a wire-like element adapted for fusion at one end to a semiconductive body, the outer wire portions consisting essentially of aluminum and containing a genetic oxide layer having a thickness between 3 and 40 microns enabling fusion of the aluminum without destruction of the layer.
- 10 2. A semiconductor device comprising a semiconductive body, and a wire-like element fused at one end to the semiconductive body, the outer wire portions consisting essentially of aluminum and containing a genetic aluminum oxide layer having a thickness between about 3 and 40 microns.
- 15 3. A device as set forth in claim 2 wherein the wire-like element comprises a core of a semiconductive material, an envelope of aluminum, and a surrounding aluminum oxide coating.
- 20 4. A device as set forth in claim 2 wherein the wire-like element comprises a core of an impurity material, an envelope of aluminum, and a surrounding aluminum oxide coating.
- 25 5. A semiconductor device comprising a semiconductive silicon body, and an aluminum wire-like element fused at one end to the semiconductive body, the outer wire portions containing a genetic aluminum oxide layer having a thickness between about 5 and 40 microns.
- 30 6. A method of making a semiconductor device comprising, providing a wire whose outer portions consist essentially of aluminum, subjecting said wire to an oxidizing treatment to provide on the aluminum portions a genetic oxide layer having a thickness enabling the aluminum to be fused without destruction of the oxide layer, and fusing an end of the said wire to a semiconductive body.
- 35 7. A method of making a semiconductor device comprising providing a wire whose outer portions consist essentially of aluminum, subjecting said wire to an oxidizing treatment to provide a genetic oxide layer having a thickness of at least about 5 microns, placing a cut end of the said wire in contact with a semiconductive body, and heating the assembly at a temperature at which the wire end fuses to the semiconductive body.
- 40 8. A method of making a semiconductor device comprising providing an aluminum wire, subjecting said wire to an oxidizing treatment to provide thereon a genetic aluminum oxide layer having a thickness between 3 and 40 microns, placing a cut end of the wire in contact with a silicon semiconductive body, and heating the assembly in an oven at a temperature above the eutectic temperature of the silicon-aluminum alloy and at which the wire end fuses to the silicon body.
- 45 9. A method as set forth in claim 8 wherein the wire is oxidized by immersing it in an oxidizing bath.

References Cited in the file of this patent

UNITED STATES PATENTS

- |           |                   |       |                |
|-----------|-------------------|-------|----------------|
| 2,840,770 | Jackson           | ----- | June 24, 1958  |
| 2,844,770 | Vessem            | ----- | July 22, 1958  |
| 2,906,932 | Fedotowsky et al. | ----- | Sept. 29, 1959 |

UNITED STATES PATENT OFFICE  
CERTIFICATE OF CORRECTION

January 2, 1962

Patent No. 3,015,761

Ludovicus Augustinus Lambertus Esseling

It is hereby certified that error appears in the above numbered patent requiring correction and that the said Letters Patent should read as corrected below.

Column 2, line 17, after "of" insert -- n-type --; line 65, for "H<sub>3</sub>PO<sub>3</sub>" read -- H<sub>3</sub>PO<sub>4</sub> --; line 68, for "(NH<sub>4</sub>)<sub>2</sub>HPO<sub>3</sub>" read -- (NH<sub>4</sub>)<sub>2</sub>HPO<sub>4</sub> --; column 3, line 9, for "C<sub>2</sub>H<sub>4</sub>H<sub>2</sub>.2H<sub>2</sub>O" read -- C<sub>2</sub>O<sub>4</sub>H<sub>2</sub>.2H<sub>2</sub>O --.

Signed and sealed this 1st day of May 1962.

(SEAL)

Attest:

ERNEST W. SWIDER

Attesting Officer

DAVID L. LADD

Commissioner of Patents